

Patented Oct. 21, 1924.

1,512,139

# UNITED STATES PATENT OFFICE.

RALPH E. SAYRE, OF NEW ROCHELLE, NEW YORK.

## CONCENTRATION OF ORES BY FLOTATION.

No Drawing.

Application filed November 24, 1923. Serial No. 676,859.

*To all whom it may concern:*

Be it known that I, RALPH E. SAYRE, a citizen of the United States, residing at New Rochelle, in the county of Westchester, State 5 of New York, have invented certain new and useful Improvements in the Concentration of Ores by Flotation; and I do hereby declare the following to be a full, clear, and exact description of the invention, such as 10 will enable others skilled in the art to which it appertains to make and use the same.

This invention relates to the concentration of ores, minerals and the like by flotation and has for its object the provision of 15 certain improvements in flotation processes.

The invention is based upon the discovery that improved results are obtained by carrying out the flotation operation in a non-acid or alkaline pulp in the presence of a heavy 20 metal xanthate, that is a heavy metal salt of xanthic acid. I have found that heavy metal xanthates, and more particularly lead xanthate, are admirable flotation agents in a non-acid or alkaline pulp. Such xanthates 25 have a marked selective action on sulfide minerals, as distinguished from gangue minerals, and cause the sulfide minerals to float readily with an attendant high recovery of the metal values. My investigations have 30 indicated that the xanthates, in a non-acid or alkaline pulp, are lacking in frothing power, so that an appropriate frothing agent, such as pine oil or terpineol should be employed in conjunction therewith in carrying 35 out the flotation operation.

The heavy metal xanthates are solid compounds, and in general are only slightly soluble in water. A heavy metal xanthate may be obtained by adding a solution of a 40 heavy metal salt to a dissolved xanthate, such for example, as potassium or sodium xanthate. In most cases, precipitation of the desired xanthate occurs immediately, and if the conditions are favorable, the yield 45 is practically quantitative as calculated on the amount of potassium xanthate used. Being the salt of a weak acid, the heavy metal xanthate may be easily hydrolyzed, and even very dilute mineral acids liberate 50 xanthic acid from it.

Free xanthic acid is an oily liquid, heavier than water, in which it is very slightly soluble and possesses a strong disagreeable odor. Xanthic acid is quite unstable, breaking up 55 spontaneously into carbon bisulfide and

alcohol. Authoritative reference books give 24° C. as the temperature at which such decomposition occurs, but my investigations have indicated that xanthic acid decomposes into carbon bisulfide and alcohol at even 60 lower temperatures.

While xanthic acid appears to have some selective action or collecting power for sulfide minerals in the flotation operation, it is in no sense so powerful and satisfactory a 65 flotation agent as the xanthates. Furthermore, owing to the instability of xanthic acid it is effective only at low temperatures, or when the flotation operation is performed immediately after its introduction into or 70 liberation in the ore pulp. Otherwise decomposition of the xanthic acid takes place and no beneficial effect in the flotation operation is obtained.

My investigations have demonstrated that 75 the beneficial effects of the xanthates as flotation agents are secured only in non-acid or alkaline mineral pulps. When a heavy metal xanthate, such for example as lead or zinc xanthate, is added to an acid mineral 80 pulp, xanthic acid is liberated. If the temperature of the pulp is much above 10° C. the liberated xanthic acid is soon decomposed into carbon bisulfide and alcohol. For these reasons, my investigations have indicated that the use of xanthates in an acid 85 pulp give very erratic, unreliable and unsatisfactory flotation results.

When the xanthate, such as lead xanthate, zinc xanthate, or the like, is used as a flotation agent in a neutral (that is non-acid) or alkaline pulp, very satisfactory flotation results are secured. Where the ore or mineral pulp is normally acid, any appropriate alkali may be used to make the pulp neutral 90 or alkaline. In this connection, satisfactory results are obtained with such alkaline agents as caustic soda, soda ash, or lime. It is preferable in general practice to add the alkaline agent to the ore or mineral prior 95 to the fine grinding which usually precedes the flotation operation. It is generally preferable to add the heavy metal xanthates to the flotation circuit prior to the final grinding of the ore or mineral.

I have found that while the heavy metal xanthate brings about a high recovery, using either lime or caustic soda in the proportions of four pounds per ton of dry ore, the use of lime is generally preferable. This 100

seems to be due to an inhibiting action on the froth when caustic soda is used, in consequence of which from 3 to 6 times the usual amount of frothing agent is required. With lime, on the other hand, the usual quantity of frothing agent suffices.

The flotation results secured, when using heavy metal xanthates as flotation agents, vary with the xanthate used. I have secured 10 most satisfactory results with lead xanthate. Flotation tests have shown that good results can be obtained when these compounds are used in the proportion of 0.1 pound per ton of dry ore or even less.

15 The following table gives some typical flotation results obtained with a number of heavy metal xanthates on ore of the Utah Copper Company assaying 1.20% copper. In each case, 500 grams of minus 40 mesh 20 ore was ground for 20 minutes in a pebble mill with 250 c. c. of water to which lime and the xanthate in the proportion of four pounds and 0.2 pounds respectively, per ton of ore, had been added. The resulting pulp 25 was diluted to about 2½ liters, a drop of terpineol was added and flotation was performed in a Callow rougher cell.

| 30 | Reagent           | Concentrate % Cu. | Tailing % Cu. | Recovery % |
|----|-------------------|-------------------|---------------|------------|
|    | Lead xanthate     | 18.0              | 0.24          | 81.1       |
|    | Zinc xanthate     | 12.8              | 0.29          | 77.1       |
|    | Iron xanthate     | 17.1              | 0.29          | 77.1       |
|    | Copper xanthate   | 16.5              | 0.36          | 71.6       |
|    | Mercury xanthate  | 12.9              | 0.40          | 68.8       |
| 35 | Chromium xanthate | 12.1              | 0.53          | 58.4       |
|    | Tin               | 13.8              | 0.28          | 78.3       |
|    | Nickel            | 16.2              | 0.41          | 67.5       |
|    | Bismuth           | 12.3              | 0.29          | 77.7       |
|    | Antimony          | 13.4              | 0.31          | 75.9       |
|    | Arsenic           | 12.5              | 0.30          | 76.9       |

40 I claim:

1. The improvement in the concentration of minerals by flotation which comprises subjecting the mineral in the form of a non-acid pulp to a flotation operation in the presence of a heavy metal xanthate.

2. The improvement in the concentration

of minerals by flotation which comprises subjecting the mineral in the form of an alkaline pulp to a flotation operation in the presence of a heavy metal xanthate.

50

3. The improvement in the concentration of minerals by flotation which comprises subjecting the mineral in the form of a pulp made alkaline by the addition of lime to a flotation operation in the presence of a heavy 55 metal xanthate.

4. The improvement in the concentration of minerals by flotation which comprises subjecting the mineral in the form of a non-acid pulp to a flotation operation in the presence of lead xanthate.

60

5. The improvement in the concentration of minerals by flotation which comprises subjecting the mineral in the form of an alkaline pulp to a flotation operation in the presence of lead xanthate.

65

6. The improvement in the concentration of minerals by flotation which comprises subjecting the mineral in the form of a pulp made alkaline by the addition of lime to a 70 flotation operation in the presence of lead xanthate.

7. The improvement in the concentration of minerals by flotation which comprises subjecting the mineral in the form of a non-acid pulp to a flotation operation in the presence of a heavy metal xanthate and a frothing agent.

75

8. The improvement in the concentration of minerals by flotation which comprises subjecting the mineral in the form of an alkaline pulp to a flotation operation in the presence of lead xanthate and a frothing agent.

80

9. The improvement in the concentration of minerals by flotation which comprises subjecting the mineral in the form of a pulp made alkaline by the addition of lime to a flotation operation in the presence of lead xanthate.

85

In testimony whereof I affix my signature.

RALPH E. SAYRE.